

May 13, 1941.

L. POLLAK

2,241,519

PHOTOGRAPHIC MATERIAL

Filed May 20, 1937

Fig. 1.



Fig. 2.



Fig. 3. EXPOSING, DEVELOPING AND PROCESSING



Fig. 4.



Inventor  
Louis Pollak  
by Michael x Michael  
Atlys.

## UNITED STATES PATENT OFFICE

2,241,519

## PHOTOGRAPHIC MATERIAL

Louis Pollak, Altrincham, Cheshire, England

Application May 20, 1937, Serial No. 143,704  
In Great Britain May 23, 1936

7 Claims. (Cl. 95—2)

My invention relates to colour photography and in particular to colour photographic negative and positive records, principally for colour motion pictures, on the subtractive principle of the kind comprising two or three superposed emulsion layers on a Celluloid or other suitable support, with or without interposed light filters. The invention also includes the method of producing and processing the photographic material.

In the production of colour photographic records it is known to employ additive and subtractive processes. The former employ a carrier of Celluloid or other transparent material provided with red, green and blue grains in mosaic or geometrical patterns, upon which a panchromatic emulsion is coated. The disadvantages of these additive processes are, considerable loss of light resulting in indefinite colours, high costs of production, unsatisfactory whites originating from overlapping of the differently coloured grains, lack of brilliancy in colours, particularly primrose, other yellow and rose tints, the difficulty of eliminating the grain effect in the projection on the screen and finally the impossibility of duplication of the original.

In the known subtractive processes three basic colour (or two basic colour combinations) separation negatives have to be made by exposure through suitable filters, which negatives may be made adaptable for still photography or cartoon films, but for moving objects such as generally form the subject matter of cinematography, the simultaneous exposure of three separation negatives can only be effected with a camera specially constructed for this purpose with splitbeam device and bi-pack. Stereoparallax and double image reflections are difficult to overcome, fully opened aperture and excessive light, so very detrimental to the comfort and the acting qualities of the performers, are required, while the definition of bi-pack images thrown on the screen at 200 to 300 enlargement results in unsharp outlines and the need to employ a fourth, i. e. black screen image.

The printing of the positives is slow and irregular, with consequently high waste production and indefinite production costs. Where print matrices from the three (two) separation negatives are made, and the positives printed by imbibition, only images of a fairly large size can be successfully made. For cinema film purposes the images are too small and the unavoidable transgression in the registration of the three (two) dye images during printing seriously affects the fine outlines and gradation of the combined

colour image when magnified on the screen. The successive three (two) printing processes from matrix to positive image carrier demand a very precisely working machine and still more perfect working material. Negatives, matrices, positive materials passing through a number of chemical and mechanical processes are bound to shrink or stretch. Matrices or wash-out-reliefs according to the Koppmann patents (pyrocatechine-developer without sodium-sulphite) or by bromoil bleaching are used, and as dye medium acid dye-stuffs, which are irregular in their application, in as much as the dye bleeds and its very slow transfer does not take place without remainder, resulting in positives, not two of which are alike in colour gradation. The transfer of basic dye-stuffs is quicker and more complete, but according to the capillar principle the matrix is bound to carry loose dye in the fine crevasses of the image, which through the pressure applied in printing will appear on the positive in blurred outlines, creating around the white objects an aureole so disturbing to the eye. The harmonising of colours, their concentration, their printing time, the correct light exposure of the negatives, the indefinite gamma values of the negatives and print matrices are factors of such intricate nature, that the slightest divergence of any of them from the theoretically perfect prescription will lead to considerable waste, and therefore unprofitable production. To avoid these difficulties systems have been evolved, in which a photographic colour element carries a plurality of superimposed layers sensitised to different colours, such elements being exposed so as to obtain images in the respective layers corresponding to the colour sensations to which the respective layer is sensitised. Quite a number of systems based on this principle have been patented with the uncertainty in the control of the various processes involved, more particularly the limitation of the penetration to each individual layer, the developing and bleaching of each layer and finally the removal of the silver halide from these layers, none of which will permit perfectly coloured images to be obtained. These images are not fast to light, they bleach out easily, and are affected by acids, even such weak reactions as the carbon-dioxide contained in the air. There are further the reversal processes, wherein the colours are contained in the layers, between which a thin clear insensitive gelatine film dyed to act as a filter is placed, and wherein the images are decolorised and reconverted to silver salt images, which are subjected to a colour de-

veloper with eventual removal of the silver from all the layers.

In all these processes real positive control is missing, they depend upon perfectly exact timing and handling, so that their success depends upon highly expert treatment. Although markings have been provided, it is exceedingly difficult to estimate correctly the time of developing and bleaching and removal of silver within the first and second top layers without affecting the lowest layer. Colour corrections are impossible and the slightest variation in the exposure will affect correct colour rendering. Finally such processes do not permit the production of positives and are therefore restricted to amateur- and mainly sub-standard films.

According to the present invention a layer consisting of a silver halide gelatine emulsion sensitised to part of the whole visible spectrum, or two such layers, sensitised to different parts of the spectrum, and the gelatine of which is so hardened as to be insoluble in warm water, has or have superposed another layer of silver halide gelatine emulsion sensitised to another part of the whole visible spectrum in which the gelatine is not hardened, in order to permit the formation of a wash-out-relief in accordance with the silver image produced, or is only hardened to the extent of still being soluble in warm water, this layer (or layers) containing a dye-forming substance enabling the formation of an image insensitive to the influence by the silver image, in a dye or colour substantially complementary to that part of the visible spectrum to which this layer is sensitized. Alternatively one of the layers of silver halide emulsion hardened and sensitised for one part of the whole visible spectrum may be arranged on the other side of the Celluloid or other support or on a separate element which is exposed simultaneously and in close contact with the double layer element recording two parts of the whole visible spectrum.

The negative is exposed in an ordinary camera and after processing is printed on a positive of similar construction, the negative recording the three primary colours, while the positive will record the three colours supplementary to those of the negative, for which a fine grain emulsion of less sensitivity is recommended. Such positive record may, however, be used for reproduction of negatives produced according to other methods, in every instance permitting the ordinary contact or optical printer to be employed.

The invention will now be more particularly described with reference to the accompanying drawing, wherein the same reference letters or characters refer to the same thing or part throughout the several views and in which:

Figure 1 is a flow-sheet of a section of a film element wherein two emulsion layers are superposed on one film base or support, in the first view before exposure, in the second view after exposure and development and in the third view after further processing;

Figure 2 is a cross section of a film element having two layers of emulsion on one side of the film base or support and one layer of emulsion on the other side;

Figure 3 is a flow-sheet of a cross section of a film element corresponding to Figure 1 with the addition of a third emulsion layer on a separate film element, the first view showing the element before development and the second view the same element after development;

Figure 4 is a section of a modified film ele-

ment where all three emulsion layers are arranged on one side of the film base or support.

In carrying the invention into effect according to one convenient manner in the production of a negative element as illustrated in Figure 1 the support or film A (hereinafter referred to as the film, although such term is to be understood to include all forms of transparent supports such as plates and the like) carries a gelatine-silver halide layer B of gelatine so hardened as not to be soluble in warm water. Superimposed upon layer B is the second gelatine-silver halide layer C the gelatine of which is not hardened and is soluble in warm water, and this layer contains an agent capable of precipitating a dyestuff or an insoluble colour-former from which in the later process through colour synthesis (coupling) a suitable dye image is formed.

Having exposed this negative element in an ordinary camera, it is desensitised, developed, fixed and washed, resulting in black silver images L and M in the respective layers as indicated in the second view of Figure 1. A bath in a solution of copper sulfate, potassium-bromide and chromic acid will bleach the silver images and harden the gelatine in correspondence with the silver image in layer C. The film is then bathed in warm water and such parts of the gelatine and the dye forming substance in layer C which have not been hardened will thereby be removed and a wash-out-relief image created.

The film is next placed in a solution containing the required dye coupling compound resulting in the formation of a dyestuff image. If, for instance, the emulsion in layer C contains an azo dye forming component, such as the water insoluble salts of naphthol-, or naphthalene- or naphthylamine- or benzidine-sulfonic or disulfonic acid compounds, a diazo-compound will convert the bleached image into a dyestuff image, for example, if amido-naphthol-disulfonic acid H or the water-insoluble salts of the same form constituents of the emulsion, a diazotised solution of dianisidine produces a blue dye image. Alternatively if the diazo coupler is contained in the emulsion, the dyestuff image will be obtained by reaction in a solution of the respective azodye forming compound. Layer B, being without a colour forming or coupling component, will remain unaffected, while both layers retain the bleached silver and copper halide images. These silver and copper halide images are converted into mordant dye images by applying a solution of thiocarbamide and a thiocyanate, such as ammonia thiocyanate and subsequently dyed in any colour with a basic dyestuff.

It is not necessary for layer C to contain strictly the red and the blue part colour. The blue part colour and the red part colour may be created by combining a blue-green with bluish-red, and this measure is made use of, amongst others, in the present invention. In both layers the mordant images are dyed bluish-red, for instance the rhodamine-B. In the outer layer C the bluegreen azo-dyestuff is present, so that by the mixing of the former with the bluish red toning of the rhodamine-B the blue part colour image P in layer C and the red part colour image R in layer B are produced, as indicated in the third view of Figure 1.

The method of the present invention may be applied to more than two layers, and its processing can be simplified by combining some of the operations into one, for instance according to the following examples:

1. The first development can be carried through, instead of with the usual known developers, with a so-called tanning developer (pyrocatechin with alkali (NaOH), without sodium-sulfite), thus eliminating the bleaching bath of copper sulfate, potassium bromide and chromic acid.

2. The dye-coupling or colour-forming compound necessary to form the dyestuff image with the colour-forming or dye-coupling component, respectively, present in the emulsion of layer C can be added to the warm water bath. Thus the colour-synthesis and the creation of the wash-out-relief image in layer C may be carried out simultaneously. The creation of the wash-out-relief must however be carried out in a subsequent bath, if for instance diazo compounds are used which are decomposed at the temperature of the warm water bath so that the diazotization must be carried out between about 0° and 10° C.

3. The development of the silver images may be done directly by means of a colour-developer, for instance, para-amino-dimethylanilin, wherein the respective dye-coupling component is added to the emulsion, which is of particular advantage, when elements having three superposed emulsion layers on one side are used.

4. The silver images may be converted by way of a chemical toning process, for instance with vanadium salts into yellow toned metal compound images. As the silver halide content in the emulsion of layer B is to be higher than in layer C, a deep-yellow part-colour image will result, while the image in layer C with a smaller silver halide content just sufficient to permit the formation of the wash-out-relief, will appear only slightly yellow-toned, which toning combined with the blue azo-dyestuff in that layer forms the bluish-green image. As the density of the dyestuff image depends upon the quantity of dye-forming substance in the emulsion and not upon the silver halide content, the smaller percentage of silver halide in layer C will not impair the correct colour representation.

5. Instead of azo, diazo- or other components capable of forming a dyestuff by way of colour synthesis in the emulsion of layer C the latter may contain ingredients which precipitate dyestuffs as colour lakes or salts insoluble in water. For instance, if a calculated quantity of barium carbonate is added to the emulsion in layer C and such layer is bathed in a solution of a dyestuff of the sulfonic-acid groups, chemical reaction will cause the formation of the insoluble barium salt of that dyestuff. Since the barium content and not the amount of solute in the dyestuff solution is responsible for the density of the dyestuff image, the dye bath and warm water bath may be conveniently combined.

6. In place of dyestuff-precipitating reagents, precipitating metal compounds, such as insoluble complex acids, phosphotungstic acid, antimonic tungstic acid, silicotungstic acid and the like according to British Patent Specifications Nos. 344,365 of September 12, 1929; 353,819 of June 24, 1930, and 430,823 of June 20, 1935, may be added to the emulsion of layer C.

7. Alternatively stable leuco compounds, esters of dyestuffs, such as benzoylacetic, acetoacetic- or cyanocetic esters, pyrazolone and others may be used, while the oxydation and warm water bath may be combined.

According to one useful modification of this invention, a film element having two superposed

emulsion layers on one side and the third emulsion layer on the other side, each sensitive to the colour sensations forming part of the visible spectrum (Figure 2), is used. The lowermost layer B is sensitized with, for instance, thiocyanin or thiopseudocyanin or erythrosin for yellow and green rays and the gelatine is hardened to withstand warm water. Superposed upon this layer, preferably with an intervening filter layer, is another layer C, containing an insoluble azo-dye-forming component, sensitised with, for instance, naphthocyanin for yellow and red rays and with the gelatine not hardened, so as to be soluble in warm water. On the reverse side of the film element A is arranged an ordinary gelatino-silver halide emulsion layer D which is hardened and only sensitive to blue rays, being preferably poor in silver and transparent.

20 After exposure in an ordinary camera, the film is desensitised, developed, fixed and washed. A solution of copper sulfate, potassium bromide and chromic acid will turn the black silver images into copper images and harden the developed portion of the gelatine. The film then passes into a bath of warm water of 25 to 30° C., in which the unhardened gelatine and the dye-forming component are removed and a wash-out-relief image created in layer C. The diazo-compound, in this instance diazotised dianisidine, to form the blue-green dyestuff by reaction with the azo-dye-forming component, for instance, amido-naphthol-disulfonic acid-H, is contained in the next following bath. In the 25 next stage the film is placed in a solution of thiocarbamide, ammonium thiocyanate and glacial acetic acid, whereby the bleached copper images are converted into mordant dye images. The film is then subjected to a waterbath, after 30 which it is placed in a solution of rhodamine-B with a slight addition of acetic acid, thereby toning the mordant dye images intensely bluish-red. After another waterbath, the film is ready to pass into the drying chamber.

45 The two superposed layers containing two of the three part-colour images, the red and the blue, are thus automatically formed, while the image in layer D on the other side of the base or support, intended for the yellow part image, is also red and as a further process in the developing machine the surface of the side carrying the emulsion layers B and C of the dried film is varnished for protection.

In another bath an oxidant, for instance a 50 weak solution of potassium permanganate with a slight addition of sulfuric acid, removes the red dyestuff of the mordant image in layer D. The film is then clarified in a waterbath and in a successive toning bath containing a yellow 55 basic dyestuff, such as acridine-yellow, thioflavin T (Schultz 6th ed. No. 618) and the like the mordant image in layer D is dyed yellow.

According to another modification of the invention, a film element having superposed two 60 emulsion layers on one side, each sensitive to the colour sensations of one part of the visible spectrum, is exposed in an ordinary camera simultaneously and in close contact with a separate film element carrying only on gelatine-silver halide emulsion sensitised to the colour sensations of the remaining part of the visible spectrum as shown in the first view of Figure 3. The lowermost layer B of the double-coated element contains a gelatine-silver halide emulsion 65 hardened to withstand warm water, sensitive to

blue rays and conveniently containing a yellow screening dyestuff. Superposed on layer B is layer C the gelatine-silver halide emulsion of which is not hardened and therefore soluble in warm water, sensitive to green and yellow rays and contains an insoluble azo-dye-forming component, such as an insoluble salt of naphthol-, or naphthalene- or napthylamine- or benzidine-sulfonic or disulfonic acid compounds, which by coupling with a diazo compound is capable of forming a red dyestuff image. Alternatively, if the emulsion is sensitised for yellow and red rays, a blue dyestuff image may be formed as previously described. The silver content in the emulsions of both layers is so chosen as to permit the formation of a weak silver image in the wash-out-relief of layer C. In place of the azo-component for the colour synthesis in layer C precipitators (lake formers) for dyestuffs or the insoluble lake combination of a leuco dyestuff may be used as previously stated.

The separate film element S, the emulsion of which is sensitive to either red and yellow or green and yellow, whichever colour sensations are not provided for in the double coated element, is developed like any ordinary black and white film (second view of Figure 3), its black silver image being converted into a mordant dye image by any known method and dyed with basic dyestuff either red or blue as required to complete the colour range of the visible spectrum. As the silver halide emulsions in the front double-coated film element are nearly transparent owing to their limited silver-content, the image of the black or separate film element S will be sharply outlined.

In a further modification of this invention the exposed film element carrying the two latent images in layers B and C is desensitised, developed and fixed in the tubular developing machine. After a tanning bath, the film passes into a warm waterbath to which the diazo coupling compound to form the dye image with the azo-dye-forming component contained in the emulsion is added, thereby simultaneously creating the wash-out-relief image and the colour synthesis therein, or alternatively, if the emulsion in layer C contains a dyestuff precipitator, the formation of an insoluble lake. The bleached silver images are then converted into mordants by means of a solution of thiocarbamide and a thiocyanide, after which they are stained with a yellow basic dye. Layer B now records the yellow part-image, while the mordant image in layer C, though slightly affected by the staining with the yellow basic dye, will register either the blue or red part colour, whichever was chosen to be produced in the above described colour synthesis. The separate film element, which is to provide the third part colour image, is treated as above described and its resulting mordant image dyed with basic dyestuff in the part colour not represented in the double coated film element. When placed in register, the two films will show the correct three part colour negative, covering the whole of the visible spectrum. Alternatively, in place of the separate element processed as above, a print copy may be made from it after development and fixing, which is converted into a wash-out-relief image and used as a print matrix, i. e. dyed in the required part colour and this dyestuff image transferred by imbibition upon one of the gelatine layers of the double coated film element, thereby completing the full range of the part colours of the visible spectrum on one element.

For reproduction in natural colours complementary to the negative record a positive element carrying three layers of fine grain gelatine-silver halide emulsion of rather less sensitivity than that selected for the negatives, superposed on one side (Figure 4), is provided, the construction of which may be conveniently arranged as follows: On a film or other transparent support is placed a hardened gelatine-silver halide emulsion layer B, which is only sensitive to blue rays, for instance a silver bromide or bromide-chloride emulsion, containing a yellow filter dyestuff or alternatively a yellow filter between layers B and C. Superposed upon layer B is layer C which consists of a gelatine-silver halide emulsion highly sensitised to green or red and hardened. Above layer C is arranged layer D containing a gelatine-silver halide emulsion not hardened, highly sensitised to red or green, whichever of the colour analysis is not used in layer C and an azo-dye forming component or dye precipitator as previously described.

The duplicating process from the negative colour records produced according to the invention, with the aid of an optical or contact printer, as used for ordinary black and white printing, may be conveniently carried out as follows: In the first part of that process, the negative colour record or records is or are projected through a strong yellow filter, such as tartrazine (Exposure Multiplication Factor 4) upon the positive element, which will produce latent images in layers C and D, without affecting layer B. These latent images are processed in a tanning developer, such as pyrocatechin and alkali (NaOH), without sodium sulfite, resulting in black silver images in each of the layers, of which the image in layer D appears tanned. In the subsequent warm water bath, to which may be added the diazo coupler or, if a precipitator is present in the emulsion of layer D a dyestuff, the developed and tanned image of layer D is converted into a dyed relief image. The film is now bathed in a solution of copper sulfate, potassium citrate and potassium ferricyanide, which turns the black silver images into mordants and is subsequently dyed in the required colour with a basic dyestuff, for instance, if dyed with rhodamine-B (Schultz 6th ed. No. 573), bluish-red images will appear in layers C and D. By further treatment in a bath containing a suitable diazo-compound the azo-dye forming component in relief image of layer D will form a blue-green azo-dyestuff image. Thus in effect the layers C and D together record the blue and red part colour images. The negative colour record is now projected upon the positive element through a blue filter. Once more developed a black silver image will appear in layer B, which may either be toned in a bath of vanadium chloride, acetic acid and potassium ferro-cyanide, or immediately after exposure treated in a yellow dye developer. The remaining silver halide in the three layers is now fixed out.

This positive processing may be reversed in its order by the projection through the blue filter being applied first and the resulting latent image in layer B developed and toned yellow in the manner described above. The projection through a yellow filter follows on, with subsequent treatment and dye image formation in layers C and D as described above, in conclusion of which the silver halide in all the three layers is removed in a fixation bath.

Instead of using the negative colour record

produced according to this invention, negatives obtained by other known processes, particularly those known under the registered trade-marks "Dufaycolor" and "Finlaychrome," may be duplicated upon positive elements in accordance with this invention, whereby the reseau or screen effect characteristic upon such negatives produced by the additive principle will be eliminated in the positive images, which, being dyestuff images, are entirely free from grain and therefore do not record the screen effect of the negative.

In order to avoid the use of the complicated and expensive colour cameras with beam splitting device or reflecting mirrors for the production of colour separation negatives, the negative colour record element according to this invention may be adopted. In this case the usual dye-transfer relief images are extracted from the exposed and processed negative and the printing process on a positive carried out by the method well known under the registered trademark "Technicolor" or any other known imbibition process.

The invention is not limited to the construction and treatment of the film described herein by way of example. It may be applied to other photographic elements such as plates and other transparent material. Films described in this invention may carry a sound track.

Various changes may be made in the details disclosed in the foregoing specification without departing from the invention or sacrificing the advantages thereof.

I claim:

1. Photographic material, particularly for colour photography, comprising a support and a plurality of light sensitive silver halide gelatine emulsion layers on this support one of said layers being sensitized to part of the visible spectrum, the gelatine in this layer being so hardened

as to be substantially insoluble in warm water, while in another of said layers, sensitized to another part of the spectrum, the gelatine is soluble in warm water and the silver halide content is smaller than in said first-mentioned layer so as to permit after normal exposure only the formation of a weak silver image by a developing treatment which produces a strong silver image in said first-mentioned layer, these two layers being attached in superimposed relation on one side of said support with the soluble layer outermost, and a colour forming substance in said soluble layer enabling the formation of an image, in a colour substantially complementary to the part of the spectrum to which this soluble layer is sensitized.

2. The photographic material of claim 1, in which another insoluble emulsion layer is arranged between the soluble and the insoluble layer mentioned.

3. The photographic material of claim 1, in which another insoluble emulsion layer is arranged on the second side of the support.

4. The photographic material of claim 1 in combination with another insoluble emulsion layer, arranged on a separate support, in close contact with the soluble layer of the first support.

5. The photographic material of claim 1, in which the gelatine in the soluble layer is partly hardened so as to still be soluble in warm water.

6. The photographic material of claim 1, in which the dye forming substance in the water-soluble layer is an azo-coupling component capable of forming, with a coupler, a dyestuff image.

7. The photographic material of claim 1, in which the colour forming substance incorporated in the soluble layer is a compound capable of producing, in this layer, insoluble precipitates from normally water soluble dyestuffs.

LOUIS POLLAK.